

1

3,524,205

PROCESS FOR THE DYEING OF SYNTHETIC POLYAMIDE FIBRES AND FABRIC FROM AN ACID DYEBAATH CONTAINING AN AMINOXIDE

Werner Langmann, Cologne-Flittard, Hellmuth Pantke, Leichlingen, Udo-Winfried Hendricks, Cologne-Stammheim, and Mathieu Quaedvlieg, Opladen, Germany, assignors to Farbenfabriken Bayer Aktiengesellschaft, Leverkusen, Germany, a corporation of Germany  
No Drawing. Filed Aug. 10, 1967, Ser. No. 659,614  
Claims priority, application Germany, Aug. 19, 1966, F 49,982

U.S. Cl. 8—172

Int. Cl. D06p 3/24

4 Claims

ABSTRACT OF THE DISCLOSURE

The process of dyeing synthetic polyamide fibres or fabric, e.g. poly-caprolactam, in an acidic aqueous dye bath in the presence of an aminoxide, e.g.



The present invention relates to a process for dyeing synthetic polyamide fibres or materials containing such fibres in an acidic aqueous dye bath; more particularly it concerns a process wherein the dyeing is carried out in the presence of aminoxides which contain an alkyl radical with at least 8 to 20 carbon atoms or an alkylaryl radical linked with the nitrogen atom directly or via bridge members.

Compounds of the following formulae can be used as aminoxides for the process of the present invention, for example:



In these formulae  $\text{R}_1$  stands for an alkyl radical with 8 to 20, preferably 12 to 18, carbon atoms,  $\text{R}_2$  and  $\text{R}_3$  independently of one another, stand for an alkyl radical with 1 to 12 carbon atoms or for the grouping  $(\text{C}_2\text{H}_4\text{O})_n\text{H}$  in which  $n$  denotes an integer from 1 to 20,  $\text{R}_4$  stands for an alkyl radical with 8 to 20 carbon atoms or for an alkylaryl radical,  $\text{R}_5$  and  $\text{R}_6$ , independently of one another, stand for alkyl radicals with 1 to 4 carbon atoms,  $\text{X}$  stands for oxygen or sulphur, and  $\text{Y}$  stands for a bivalent alkylene radical with 2 or 3 carbon atoms which may be substituted by methyl or hydroxyl, while  $m$  denotes an integer from 1 to 10.

Alkyl radicals represented by  $\text{R}_1$  are, for example, decyl, dodecyl, 2,2-dimethyldecyl, isotridecyl, hexadecyl and octadecyl; alkyl radical represented by  $\text{R}_2$  and  $\text{R}_3$  are, for example, methyl, ethyl, propyl, octyl and dodecyl;

2

alkyl or alkylaryl radicals represented by  $\text{R}_4$  are, for example, decyl, dodecyl, 2,2-dimethyldecyl, 2,2,4,6,6-pentamethyl-heptyl-(4), isotridecyl, hexadecyl, octadecyl, iso-octyl-phenyl and isononyl-phenyl; and alkyl radical represented by  $\text{R}_5$  and  $\text{R}_6$  are, for example, methyl, ethyl, isopropyl and butyl, while  $\text{Y}$  stands, for example, for the radicals  $-(\text{CH}_2)_2-$ ,  $-(\text{CH}_2)_3-$ ,



or  $-\text{CH}_2-\text{CH}(\text{OH})-\text{CH}_2-$ .

Aminoxides corresponding to the above Formula I wherein  $\text{R}_2$  and  $\text{R}_3$  stand for alkyl radicals, can be obtained, for example, by treating the tertiary amines from which they are derived with hydrogen peroxide.

Aminoxides corresponding to the Formula I wherein  $\text{R}_2$  and/or  $\text{R}_3$  stand for the grouping  $(\text{C}_2\text{H}_4\text{O})_n\text{H}$ , can be obtained, for example, by treating the reaction products of ethylene oxide on appropriate primary or secondary amines with hydrogen peroxide.

Aminoxides corresponding to the Formula II wherein  $\text{Y}$  stands for  $-(\text{CH}_2)_2-$ , can be obtained, for example, by preparing from the reaction product of 1 mol ethylene oxide on 1 mol of an alcohol, mercaptan or alkylphenol containing the radical  $\text{R}_4$ , the alkali metal or ammonium salts of the acidic sulphuric acid ester, reacting these with appropriate secondary amines in the presence of strong bases and then treating the resultant ether amines with hydrogen peroxide.

Compounds of the Formula II wherein  $\text{Y}$  stands for  $-(\text{CH}_2)_3-$  or for  $-\text{CH}_2-\text{CH}(\text{CH}_3)-\text{CH}_2-$  can be obtained, for example, by reacting alcohols, mercaptans or alkylphenols containing the radical  $\text{R}_4$  with acrylonitrile or methacrylonitrile, reducing the resultant cyanoethyl or cyanopropyl ethers to form the primary ether amines, converting these into tertiary ether amines by alkylation, and then treating the tertiary ether amines with hydrogen peroxide.

Compounds of the Formula II wherein  $\text{Y}$  stands for  $-\text{CH}_2-\text{CH}(\text{OH})-\text{CH}_2-$ , can be obtained, for example, by reacting alcohols, mercaptans or alkylphenols containing the radical  $\text{R}_4$  with epichlorohydrin, reacting the resultant glycidyl ethers with appropriate secondary aliphatic amines and then treating the resultant tertiary ether amines with hydrogen peroxide.

The compounds of the Formula III can be obtained according to analogous methods by using, instead of the alcohols, mercaptans or alkylphenols containing the radical  $\text{R}_4$  themselves, the appropriate reaction products thereof with ethylene oxide.

Dyestuffs which can be used in the process according to the invention are, for example, substantive dyestuffs, acid dyestuffs and 1:2 metal complex dyestuffs.

The necessary amounts of aminoxides can easily be established by preliminary experiments; in general, 0.1 to 5 parts by weight aminoxide per 1 part by weight of dyestuff will prove sufficient. Dyeing of the synthetic polyamide fibres can then be carried out in the usual manner.

With the aid of the process according to the invention it is possible to obtain very level dyeings on synthetic polyamide fibres, for example, fibres made of poly-caprolactam, of the polycondensation product of hexamethylene diamine and adipic acid or of the polycondensation product of  $\omega$ -amino-undecanic acid, as well as on materials containing such fibres, such as fabrics or knitted fabrics. This is surprising, because the risk of an uneven dyeing which exists when dyeing synthetic polyamides, due to the differences in affinity, titre and thread tension which are always present, cannot be satisfactorily obviated by the use of levelling agents such as have hitherto been used for dyeing of synthetic fibres.

The following examples serve to illustrate the invention without, however, limiting its scope; the parts given are parts by weight.

## EXAMPLE 1

0.05 part of the dyestuff Colour Index, 2nd edition, No. 29,035 and 0.008 part aminoxide of the formula



are dissolved in 5 parts of water; in addition, 0.05 part of the dyestuff Colour Index No. 23,150 and 0.131 part of the above aminoxide are dissolved in 5 parts of water, and 0.025 part of the dyestuff Colour Index No. 22,155 and 0.015 part of the above aminoxide are dissolved in 2.5 parts of water. The three solutions are then stirred into 3000 parts of water which was adjusted with 85% formic acid to a pH value of 3 and to which 0.5 part of the above aminoxide had been added. 100 parts of knitted goods made of poly- $\epsilon$ -caprolactam threads are introduced into the dyebath thus prepared and heated to 30–40° C., the dyebath is heated to 90–100° C. in the course of 30 minutes, and kept at this temperature for a further 30 to 60 minutes. The knitted goods are finally rinsed in water and then dried. A very level green dyeing of good fastness to light and wet processing is obtained.

The aminoxide used was prepared as follows:

342 parts of the reaction product of 3 mol ethylene oxide on 1 mol isotridecyl alcohol were mixed dropwise at 10–20° C. with 127 parts chlorosulphonic acid, the mixture was stirred for 1 hour at 20–30° C. and subsequently added at 20–35° C., while cooling, to a solution of 140 parts sodium hydroxide in 600 parts of water. The resultant reaction mixture was subsequently mixed with 170 parts of a 40% aqueous dimethylamine solution and heated in an autoclave at 160–180° C. for 8 hours. The reaction product was subjected to phase separation at 80–90° C. The lower phase was removed, the upper phase was stirred hot with 150 parts of water. The resultant mixture was again subjected to phase separation; the lower phase was removed, the upper phase was then freed from water at 80–90° C. in a vacuum. 111 parts of the tertiary ether amine so obtained were dissolved in 50 parts ethanol and mixed dropwise at 60–65° C. with 45 parts of 30% hydrogen peroxide. The mixture was subsequently stirred at the same temperature for 6 hours. The unreacted hydrogen peroxide was destroyed by suspending a platinum foil in the mixture. The aminoxide formed was then freed from ethanol and water in a vacuum at 60–70° C.

## EXAMPLE 2

0.5 part of the dyestuff Colour Index No. 23,150 and 1.6 parts of the aminoxide of the formula



are dissolved in 50 parts of water; in addition, 1 part of the dyestuff Colour Index No. 29,035 is mixed with 0.2 part of the above aminoxide and the mixture is dissolved in 100 parts of water. The two solutions are stirred into 2850 parts of water which has been adjusted to a pH value of 3 by means of 85% formic acid. 100 parts of knitted goods made of poly- $\epsilon$ -caprolactam threads are then dyed in the dyebath so prepared in the manner described in Example 1. A level green dyeing is again obtained.

The aminoxide used was prepared as follows:

213 parts N,N-dimethyl-dodecylamine were dissolved in 300 parts ethanol and mixed dropwise at 50–55° C. 75

with 45 parts of 30% hydrogen peroxide. The mixture was subsequently stirred at this temperature for 5 hours. The excess hydrogen peroxide was destroyed by suspending a platinum foil in the mixture. The aminoxide formed was then freed from ethanol and water in a vacuum at 60–70° C. and recrystallised from ethyl acetate.

We claim:

1. A process for dyeing synthetic polyamide fibers or fabrics in an acidic aqueous dyebath comprising incorporating into said dyebath an aminoxide selected from the group consisting of



wherein

$\text{R}_1$  is an alkyl group of 8 to 20 carbon atoms;  $\text{R}_2$  and  $\text{R}_3$ , independently, are alkyl groups of 1 to 12 carbon atoms or  $(\text{C}_2\text{H}_4\text{O})_n\text{H}$  in which  $n$  is an integer from 1 to 20;

$\text{R}_4$  is an alkyl or an alkylaryl group of 8 to 20 carbon atoms;

$\text{R}_5$  and  $\text{R}_6$ , independently, are alkyl groups with 1 to 4 carbon atoms;

$\text{X}$  is oxygen or sulphur; and  $\text{Y}$  is an unsubstituted or a substituted bivalent alkylene radical with 2 or 3 carbon atoms wherein the substituents are methyl or hydroxyl; and

$m$  is an integer from 1 to 10.

2. The process of claim 1 wherein the aminoxide has the formula



3. The process of claim 1 wherein the aminoxide has the formula



55 4. The process of claim 1 wherein the aminoxide has the formula



## References Cited

## UNITED STATES PATENTS

|           |         |               |       |      |   |
|-----------|---------|---------------|-------|------|---|
| 2,074,380 | 3/1937  | Flett         | ----- | 8-85 | X |
| 2,220,834 | 11/1940 | Bruson et al. | ----- | 8-85 | X |
| 2,940,815 | 6/1960  | Taras         | ----- | 8-85 | X |

70 GEORGE F. LESMES, Primary Examiner

T. J. HERBERT, Jr., Assistant Examiner

UNITED STATES PATENT OFFICE  
CERTIFICATE OF CORRECTION

Patent No. 3,524,205 Dated August 18, 1970

Inventor(s) Werner Langmann, et al.

It is certified that error appears in the above-identified patent and that said Letters Patent are hereby corrected as shown below:

| <u>Column</u> | <u>Line</u>      | <u>Error</u>                                                                                                                                                                                             |
|---------------|------------------|----------------------------------------------------------------------------------------------------------------------------------------------------------------------------------------------------------|
| 4             | 1                | "45 parts" should read --- 125 parts ---                                                                                                                                                                 |
| 4             | Claim 1<br>20-25 | "-Y-N" should read --- -Y-N ---<br>  |

SIGNED AND  
SEALED  
NOV 10 1970

(SEAL)

Attest:

Edward M. Fletcher, Jr.  
Attesting Officer

WILLIAM E. SCHUYLER, JR.  
Commissioner of Patents